

## UNITED STATES PATENT OFFICE

2,206,278

## TEXTILE AND OTHER MATERIALS

Henry Dreyfus, London, England

No Drawing. Application May 5, 1937, Serial  
No. 140,897. In Great Britain May 14, 1936

10 Claims.

(Cl. 8—61)

This invention relates to textile and other products containing titanium dioxide and to an improved form of titanium dioxide particularly suitable for incorporation in artificial silks and other artificial products, for example films, moulded objects and the like.

Artificial silk having a low lustre is extensively manufactured with the aid of titanium dioxide. A small proportion of this material is incorporated in the spinning solution from which the artificial silk is formed. Another method of producing an artificial silk of low lustre is to incorporate titanium dioxide or hydrated titanium dioxide in the already spun artificial silk, e. g. by interaction of suitable reagents on the material, or by treating the material with an aqueous dispersion of titanium dioxide. It has been found, however, that when artificial silks containing titanium dioxide are coloured the colourations are in general not so fast to light as those yielded by the same dyestuffs upon similar materials free from titanium dioxide. This lack of fastness to light is particularly noticeable while the material is wet. Further, artificial silk containing titanium dioxide frequently loses strength much more rapidly when exposed to light than similar artificial silk free from titanium dioxide.

According to the present invention these undesirable effects of titanium dioxide are minimized by associating or treating it with a compound of manganese, iron, cobalt, nickel or copper. These elements are those having atomic weights ranging from that of manganese to that of copper. The titanium dioxide may be treated with the metal compound or a mixture of the metal compounds before the titanium dioxide is incorporated in the artificial silk or other material. Again, the artificial silk or other material containing the titanium dioxide may be treated with the metal compound or a mixture of the metal compounds and either before, during, or after any colouring of the material.

If desired, the treatment of a textile or other product with the metal compound may precede or be carried out simultaneously with the incorporation of titanium dioxide in the material or as a step in a process of effecting such incorporation. Moreover, a cellulose ester or other substance may be treated with the metal compound prior to conversion into filaments, e. g. while in the form of a spinning or film-forming solution, and before or after incorporation of titanium dioxide therewith.

Conveniently water-soluble compounds of the metals are employed and they may be salts of

the metals with acids or they may be compounds in which the metal forms part of an anion. Examples of suitable salts are the sulphates, chlorides, or acetates of the aforementioned metals.

The treatment or association of the titanium dioxide with the metal compound is applicable in the case of natural textile fibres containing titanium dioxide, for example natural silk, in which titanium dioxide has been incorporated. It is, however, of special value in the case of artificial silk and other artificial products containing titanium dioxide. For example, the new process may be applied in the case of regenerated cellulose artificial silk, foils, or films containing titanium dioxide, or artificial silk, films, foils, plastics and the like containing titanium dioxide and having a basis of cellulose acetate or other cellulose ester or ether.

The titanium dioxide or material containing it may be treated with an aqueous solution containing one or more of the aforementioned compounds. For example, titanium dioxide sufficiently finely sub-divided to render it suitable for incorporation in an artificial silk spinning solution may be heated or boiled with a 0.1 to 5%, e. g. 0.3 to 0.5%, aqueous solution of copper sulphate or other of the metal compounds referred to above. Again, a textile material, for example an artificial silk containing titanium dioxide, may be heated with a dilute aqueous solution of copper sulphate or other of the above-mentioned metal compounds. Such a solution may, for example contain .05 to 1% of the copper sulphate or other compound.

If desired the solutions of the metal compounds may contain an acid, for example formic acid, acetic acid, or other organic acid. The amount of acid used may be about half the weight of the metal salt.

When treating textile materials, foils, or the like containing titanium dioxide, the treatment liquid may contain a swelling agent for the cellulose acetate or other material forming the basis of the textile, foil or the like, in order to facilitate penetration of the material by the treatment liquid.

After treatment with the aqueous solution the titanium dioxide or material containing it may be washed. The material may then be dried, or further processed without drying, as may be convenient. For example, in the case of a textile material containing titanium dioxide, the wet material may be dyed without intermediate drying.

If desired the titanium dioxide or other mate-

rial may be subjected to a treatment to ensure the fixation of an oxide, hydroxide, or other water-insoluble compound of the metal in the material. For example suitable reagents may be allowed to interact in the presence of the titanium dioxide so as to form an oxide or hydroxide of the metal on the titanium dioxide. For instance finely divided titanium dioxide may be heated with an aqueous solution of a salt of one of the aforementioned metals and an aqueous solution of an alkali slowly added in sufficient quantity to precipitate an oxide or hydroxide of the metal on the titanium dioxide.

Other methods of associating with the titanium dioxide a compound or compounds of the manganese or other metal may, however, be employed. For example the titanium dioxide may merely be intimately mixed with the compound of the metal in question. For instance an aqueous paste of titanium dioxide may be well ground with an aqueous paste of an oxide or hydroxide of the manganese, copper or other metal, the mixture being thereafter dried if desired.

The compound of manganese, copper or other metal may be employed in quite small proportion, for example a proportion of the order of .05 to 5%, e. g. .5 to 2%, based on the weight of the titanium dioxide.

The new process enables improved results as regards fastness to light to be obtained when materials containing titanium dioxide are coloured with dyestuffs of widely varying type. For example the improvement is particularly good in the case of water-soluble azo dyestuffs having a substantive affinity for regenerated cellulose. Again, the dyestuffs may be azo dyes, soluble or insoluble in water, having a direct affinity for cellulose acetate. Other classes of dyes the colourations of which on textile materials containing titanium dioxide may be improved by the new process are the amino-anthraquinone dyestuffs having direct affinity for cellulose acetate, especially those dyestuffs yielding violet, blue or green shades on this material. The improvement is particularly good in the case of dyeings made with 1,4-diamino-anthraquinone or 1,4-amino-oxy-anthraquinone and their substitution products, for example 1,4-di-(alkylamino)-anthraquinone. An improvement may be obtained even in the case of those dyestuffs normally regarded as having a very high degree of fastness, for example vat dyestuffs, e. g. those of the Indigold series, and the water-insoluble azo dyestuffs produced on the fibre, for example those produced by coupling diazotised amines with  $\beta$ -naphthol, arylamides of 2:3-oxy-naphthoic acid, or diacyl-acetyl derivatives of aromatic diamines.

The following examples illustrate the invention but are not to be regarded as limiting it in any way:

#### Example 1

Finely divided titanium dioxide is heated for 30 minutes at 85 to 90° C. with 20 times its weight of an aqueous solution containing 4 grams per litre of copper sulphate and 1.5 grams per litre of formic acid. The titanium dioxide is then filtered off, washed and dried.

For the production of artificial silk of low lustre 2 parts of titanium dioxide treated as above are incorporated in 400 parts of a 25% solution of cellulose acetate in acetone and the solution thereafter spun into filaments by dry spinning methods. Shades yielded on this artificial silk with, for example, 1,4-di-(methylamino)-anthra-

quinone, are of much better fastness to light than those on similar artificial silk made with untreated titanium dioxide.

The copper sulphate in this example may be replaced by an equal quantity of manganese sulphate ( $MnSO_4$ ), cobalt sulphate or nickel sulphate.

#### Example 2

A fabric of cellulose acetate yarns having a low lustre due to the presence of titanium dioxide therein is treated for one hour at 85° C. with an aqueous solution containing .5% of copper sulphate and .2% of formic acid. The material is well washed and is then dyed with 1,4-di-(methylamino)-anthraquinone. In this way a blue shade is obtained which is much faster to light than that obtained when the treatment with copper sulphate is omitted.

The copper sulphate in this example may be replaced by an equal quantity of nickel sulphate or cobalt sulphate or manganese sulphate ( $MnSO_4$ ).

Having described my invention, what I desire to secure by Letters Patent is:

1. Process for improving the light-fastness of colored artificial textile materials containing titanium dioxide, which comprises associating the titanium dioxide with a compound of a metal selected from the group consisting of manganese, iron, cobalt, nickel and copper, and incorporating the titanium dioxide product so produced into the artificial textile materials.

2. Process for improving the light-fastness of colored artificial textile materials having a basis of cellulose acetate and containing titanium dioxide, which comprises associating the titanium dioxide with a compound of a metal selected from the group consisting of manganese, iron, cobalt, nickel and copper, and incorporating the titanium dioxide product so produced into the artificial textile materials having a basis of cellulose acetate.

3. Process for improving the light-fastness of colored artificial textile materials having a basis of cellulose acetate and containing titanium dioxide, which comprises associating the titanium dioxide with a compound of a metal selected from the group consisting of manganese, iron, cobalt, nickel and copper, the proportion of such metal compound being from 0.05 to 1% on the weight of the titanium dioxide, and incorporating the titanium dioxide product so produced into the artificial textile materials having a basis of cellulose acetate.

4. Process for improving the light-fastness of colored artificial textile materials containing titanium dioxide, which comprises subjecting the artificial materials containing titanium dioxide to the action of an aqueous medium containing a compound of a metal selected from the group consisting of manganese, iron, cobalt, nickel and copper.

5. Process for improving the light-fastness of colored artificial textile materials having a basis of cellulose acetate and containing titanium dioxide, which comprises subjecting artificial textile materials having a basis of cellulose acetate and containing titanium dioxide to the action of an aqueous medium containing a compound of a metal selected from the group consisting of manganese, iron, cobalt, nickel and copper, and a swelling agent for the cellulose acetate.

6. Process for improving the light-fastness of colored artificial textile materials having a basis

of cellulose acetate and containing titanium dioxide, which comprises subjecting artificial textile materials having a basis of cellulose acetate and containing titanium dioxide to the action of an aqueous medium containing a compound of a metal selected from the group consisting of manganese, iron, cobalt, nickel and copper, in an amount equal to from 0.05 to 1% on the weight of the titanium dioxide, and a swelling agent for the cellulose acetate.

7. Process for improving the light-fastness of colored artificial textile materials having a basis of cellulose acetate and containing titanium dioxide, which comprises associating the titanium dioxide with copper sulphate, and incorporating the titanium dioxide product so produced into the artificial textile materials having a basis of cellulose acetate.

8. Process for improving the light-fastness of colored artificial textile materials having a basis of cellulose acetate and containing titanium dioxide, which comprises associating the titanium

dioxide with manganese acetate, and incorporating the titanium dioxide product so produced into the artificial textile materials having a basis of cellulose acetate.

9. Process for improving the light-fastness of colored artificial textile materials having a basis of cellulose acetate and containing titanium dioxide, which comprises subjecting artificial textile materials having a basis of cellulose acetate and containing titanium dioxide to the action of an aqueous medium containing copper sulphate and a swelling agent for the cellulose acetate.

10. Process for improving the light-fastness of colored artificial textile materials having a basis of cellulose acetate and containing titanium dioxide, which comprises subjecting artificial textile materials having a basis of cellulose acetate and containing titanium dioxide to the action of an aqueous medium containing manganese acetate and a swelling agent for the cellulose acetate.

HENRY DREYFUS